

# UNITED STATES PATENT OFFICE.

PERCY A. E. ARMSTRONG, OF LOUDONVILLE, NEW YORK, ASSIGNOR TO LUDLUM STEEL COMPANY, A CORPORATION OF NEW JERSEY.

## VANADIUM-CONTAINING IMPACT-TOOL FOR HOT WORK.

1,388,157.

Specification of Letters Patent. Patented Aug. 23, 1921.

No Drawing.

Application filed April 10, 1919. Serial No. 289,150.

To all whom it may concern:

Be it known that I, PERCY A. E. ARMSTRONG, a subject of the King of Great Britain, and a resident of Loudonville, 5 county of Albany, State of New York, have invented certain new and useful Improvements in Vanadium-Containing Impact-Tools for Hot Work, of which the following is a specification.

10 My invention relates to impact tools, such as drop forging dies, rivet sets, bull dies, and generally to impact tools which are intermittently subjected to heavy impact stresses and to comparatively high heat, as in drop forging work, riveting up hot rivets and the like.

In making impact tools for hot work, such as above referred to, having a composition within the following range:—carbon about .30-.60%, manganese about .30-1%, chromium about 1.0-1.75%, nickel about 3.5-5.0%, the remainder iron, with small proportions of impurities present in steel, as silicon, sulfur, phosphorus, copper, etc., I have found that such steel is air hardening 25 and is well adapted for such tools as drop forging dies and the like, where they are not very large, or where the impact stresses are not unduly great, or the reversals of stress are not frequent. For such work, impact 30 tools containing vanadium are preferable, but I have found that when tools are made of alloy steel within the range of composition above referred to, and vanadium is included therewith, without other change than the inclusion of vanadium, the material, which has good air hardening qualities prior to inclusion of vanadium therewith no longer has such excellent air hardening qualities, and is not so well adapted for tools for the purposes 35 referred to, as is the case with material having better air hardening qualities.

I have found that vanadium may be included to advantage and an alloy steel obtained, which is stronger dynamically and 45 better adapted to stand up under heavy impact work on hot metal as in drop forging, for example, if the proportion of nickel is increased, while the chromium content is kept about as before, or, if, keeping the 50 nickel about as before, the chromium content is increased, or if the increase is distributed between the nickel and chromium in about the relative proportion given below.

A typical illustrative example falling 55 within the composition range first above re-

ferred to contains carbon about .35%, chromium about 1.25%, and nickel about 4.75%, the rest iron, with small proportions of impurities such as already referred to.

If impact tools such as described are made 60 of this composition, and vanadium included therewith to the extent of about .25%, which is a desirable proportion, it will be found that they have no longer such excellent air hardening qualities. I have found that, in 65 order that they shall have desirably good air hardening qualities and be well adapted for the work to which they are to be put, satisfactory results may be obtained by increasing the nickel to about 5-6%, or the chromium to about 2%, or the increase may be distributed between the nickel and the chromium in about the same relative proportion 70 for each.

The following examples are typical of 75 composition for vanadium containing impact tools of the class described, but it is to be understood that these examples are given for illustration and for affording a clear understanding of my invention only, and not for limitation of the invention, as there may be more or less variation away from the precise figures given and, as already stated, the increase may be distributed between the nickel and the chromium, if desired. The percentages 80 given are by weight:—

### Example 1.

|                                                              |         |
|--------------------------------------------------------------|---------|
| Carbon about                                                 | .35%    |
| Manganese about                                              | .40% 90 |
| Chromium about                                               | 1.25%   |
| Nickel about                                                 | 6.0 %   |
| Vanadium about                                               | .25%    |
| The rest iron with small proportions of impurities as above. | 95      |

### Example 2.

|                                                             |           |
|-------------------------------------------------------------|-----------|
| Carbon about                                                | .35%      |
| Manganese about                                             | .40%      |
| Chromium about                                              | 2.0 % 100 |
| Nickel about                                                | 4.75%     |
| Vanadium about                                              | .25%      |
| The rest iron with small proportion of impurities as above. | 105       |

Impact tools for hot work, made of materials such as described, have excellent air hardening qualities, and withstand great impact stresses, standing up well in heavy work, such as making large drop forgings or other 110

heavy impact work on hot metal, or where the stress reversals are frequent.

I claim:

1. Impact tools for hot work of air hardening alloy steel, containing: carbon about .30-.60%, manganese about .30-1%, chromium about 1-1.75%, nickel about 5-6%, and also containing vanadium and the greater part of the remainder iron.
- 5 2. Impact tools for hot work of air hard-

ening alloy steel, consisting substantially of: carbon about .35%, manganese about .40%, chromium about 1.25%, nickel about 6%, vanadium about .25%, and the greater part of the remainder iron.

In testimony that I claim the foregoing I hereto set my hand, this 7th day of April, 1919.

15 PERCY A. E. ARMSTRONG.